

**1**

2,906,697

**HYDROREFORMING AND REACTIVATION OF CATALYST WITH AN OXYGEN CONTAINING GAS**

George C. Hall, Springdale Township, Allegheny County, Robert E. Kline, Penn Township, Allegheny County, and Robert C. Zabor, Ross Township, Allegheny County, Pa., assignors to Gulf Research & Development Company, Pittsburgh, Pa., a corporation of Delaware

No Drawing. Application October 11, 1954  
Serial No. 461,644

**5 Claims. (Cl. 208—136)**

This invention relates to a catalytic process for the treatment of hydrocarbons to convert them to more valuable products. More particularly, the invention relates to a process for the catalytic reforming of hydrocarbons of the naphtha or gasoline boiling range to increase the value of such hydrocarbons as components of fuels for internal combustion engines.

The petroleum industry for years has been faced with a demand for gasolines of progressively higher anti-knock quality. For some time refiners have met the demand with catalytic cracking supplemented by processes such as thermal reforming, polymerization, alkylation, etc. However, catalytic cracking is limited in its ability to upgrade the whole refinery gasoline pool. The other processes have had various economic drawbacks. The continued demand for gasolines of still higher octane ratings for use in high compression automotive engines forced the refiners to seek a new way of upgrading low octane stocks. In recent years a type of process has been developed that, when coordinated with the other refinery operations, offers economic advantages for most refiners over any other process for improving the anti-knock properties of stocks such as straight run and natural gasolines. The process we refer to is catalytic reforming in the presence of hydrogen, or "hydroreforming" as it is commonly called.

Its economic advantages have caused hydroreforming to be widely adopted and it has become one of the most important of refining processes. Several variations of the hydroreforming process are now in use. They vary somewhat in operating conditions and in the particular type of catalyst used. They have in common the fact that a gasoline or naphtha fraction is contacted with a catalyst in the presence of a large amount of hydrogen at a temperature above about 750° F. and usually at an elevated pressure. The treatment results in chemical conversion of components of the charge to materials of better anti-knock properties but without a great change in average molecular weight of the charge. A number of chemical reactions can take place in the hydroreforming process. These include (1) conversion of cyclopentane with methyl side chains to cyclohexane; (2) conversion of cyclohexane to aromatics with a large yield of hydrogen; (3) cracking of higher molecular weight paraffins; (4) hydrogenation of olefins formed as intermediate cracking products; (5) conversion of sulfur compounds to hydrogen sulfide; and (6) isomerization of normal paraffins to branched-chain paraffins. The product in general contains a higher proportion of aromatics and isoparaffins than the charge and usually has a slightly lower average molecular weight than the charge.

**2**

The competition to produce high octane gasolines has caused the process of hydroreforming to be studied in all details to find ways of increasing the yield and quality of the gasoline product. Many improvements have been made in the process since its first development. The present invention is especially significant because it provides improvement in a most important refining process that has already been brought in the prior art to a high state of efficiency.

10 Broadly, our invention pertains to an improvement in hydroreforming processes which use catalysts containing molybdenum or its oxides. The process of the invention is based on the discovery that a particular combination of catalyst reduction technique and on-stream conditions improves the results of the process, as compared with prior art hydroreforming, by producing a gasoline product of higher yield and/or of higher octane rating. The exact reasons for the improvement are not known with certainty but it is believed that the process of the invention renders the catalyst more selective for the reactions of hydroreforming that are most important for raising octane rating, for example, the aromatization of naphthenes and the isomerization of straight-chain paraffins, without excessively increasing the activity for reactions such as cracking that reduce liquid yield.

20 We have discovered, in accordance with the invention, that by reducing the reforming catalyst with hydrogen that contains a minor amount of an oxygenic gas such as steam, oxygen or carbon dioxide and then using this catalyst in an on-stream hydroreforming operation with hydrogen that is substantially free of such oxygenic gases, an unexpected improvement in yield-octane relationship of the product occurs. The enhancement of the catalyst activity by our reduction procedure remains in effect for 25 a considerable time and produces the advantages of the invention for the usual throughput period with the molybdenum catalyst.

30 The hydroreforming process of our invention is most suitable for upgrading low octane stocks such as natural or casing-head gasolines and straight-run naphthas or 35 gasolines. Natural gasoline is the volatile product obtained by the recovery of normally liquid hydrocarbons from natural gas by a process such as absorption. Straight-run gasolines are produced by fractionation of crude petroleum oil. The charge stocks for our process can also be blends of these types of stocks or blends with naphthas obtained from other processes such as thermal or catalytic cracking. Our process shows an improvement in octane-yield relationship over conventional hydroreforming whether the charge stock is predominantly 40 paraffinic or naphthenic.

45 The catalyst of our process is a molybdenum oxide type of reforming catalyst. The molybdenum oxide can be used alone but preferably is deposited on a support or carrier. Suitable carriers include activated alumina, alumina gels, peptized alumina gels, silica gels, silica-alumina gels, aged or deactivated silica-alumina cracking catalysts, silica-magnesia gels, magnesia, titania, bauxite and the like. A preferred support consists of alumina 50 stabilized with about 5 percent by weight silica. Although molybdenum is an essential element, other reforming catalyst metals or oxides, for example, cobalt and nickel, can be present in the catalyst.

55 Our process can be carried out in any of the systems for catalytic contact that are suitable for reforming. For

example, the catalyst can be in pelleted or granular form in a stationary fixed bed. It can also be in a finely divided or powdered form in a fluidized bed. The fluidized bed can be either a fixed fluid bed or a moving fluid bed. In a fixed bed system, either of the fluid or stationary type, the catalyst is kept in the same vessel for all cycles of the process, that is, for the on-stream period and for the regeneration and reduction. In the moving fluid bed the catalyst is continuously transported from the hydro-reforming vessel to other zones for regeneration and/or hydrogen reduction.

In discussing the range of operating conditions for our process we will deal with the reduction stage first. In general, the reduction can be carried out at temperatures from about 850° F. to about 1200° F. A temperature between about 1000° F. and 1100° F. produces the best results. However, the lower temperatures have the advantage of being closer to temperatures preferred for the on-stream hydroreforming stage. If the reduction and on-stream temperatures are the same, loss of time for cooling the catalyst before placing it on-stream can be avoided.

The other operating conditions of the reduction stage can vary considerably. The pressure can range from atmospheric to about 2000 pounds per square inch. (This is gauge pressure, as are the other pressures mentioned in the specification and claims.) It is advantageous to reduce the catalyst at either the pressure used during regeneration or the pressure used during the on-stream stage. The linear velocity of the reducing gas can vary considerably. We have found that rates of from about 0.01 to 1.0 foot per second give good results in a fluid bed system. In general, a reduction period of from about 0.1 to 5.0 hours is sufficient. In a moving bed fluid catalyst system the reduction can take place while the oxidized catalyst is being transported from the regenerator to the reactor by a stream of hydrogen. As we have indicated, the most important feature of the reduction stage of our process is the use of hydrogen that contains a minor amount of an oxygenic gas selected from the group consisting of steam, oxygen and carbon dioxide.

When steam is used as the oxygenic substance for mixing with the reducing hydrogen, a concentration of from 0.5 to 10 or 15 mol percent or even higher will produce the advantages of the invention. Our best results are obtained with steam concentrations of from 0.5 to 5 mol percent, based on the hydrogen. The other oxygenic substances should be used in concentrations equivalent to these steam concentrations. For an equivalent effect, oxygen and carbon dioxide can be used in one-half the mol percent concentration used for steam. If oxygen is used, care should be taken that its concentration in the hydrogen does not exceed the explosive limit.

After the reduction stage of our process, the catalyst is used for hydroreforming. The processing conditions can vary considerably, depending on the stock being treated and the balance of octane rating and yield of product desired. The most significant feature of the on-stream stage of our process is that the charge, that is, the mixture of hydrocarbons and hydrogen with which the catalyst is contacted, is substantially free of oxygenic substances.

The processing conditions for the on-stream hydroreforming stage of our process can be as follows: The temperature is above about 750° F. and preferably from about 850° F. to 1100° F. The pressure can range from atmospheric pressure to high pressures of the order of 2000 pounds per square inch. Pressures of from 50 to 500 pounds per square inch are preferred. The space velocity can be from about 0.25 to 10.0 liquid volumes of hydrocarbon per hour per volume of catalyst (based on densely packed catalyst volume). Generally, a space velocity of about one-half to three vol./vol./hour is preferred. The hydrogen concentration, or hydrogen to naphtha ratio, should be at least about 500 standard

cubic feet of hydrogen per barrel of liquid hydrocarbon charge (42 U.S. gallons) and not more than about 20,000 s.c.f. per barrel. At the start of the process it may be necessary to supply the hydrogen from an outside source.

5 However, the dehydrogenation that occurs in hydroreforming will usually produce enough hydrogen so that the hydrogen requirements can be met by recycle from the product.

Having described the general and preferred ranges of 10 conditions for our process, we will now describe some actual hydroreforming runs that we have carried out by the method of our invention and by a conventional hydroreforming technique, using the same naphtha charge stock for all runs. The results of these runs offer a comparison of the different methods and show the superiority 15 of our process over the conventional process.

The charge stock in this series of runs was a straight-run naphtha from a Kuwait crude oil. The naphtha was highly paraffinic and had a very low octane rating. The 20 inspection data for this naphtha are as follows:

#### KUWAIT NAPHTHA INSPECTION DATA

|                                               |       |
|-----------------------------------------------|-------|
| Gravity, ° API                                | 52.6  |
| Sulfur, wt. percent                           | 0.109 |
| 25 Reid vapor pressure, lbs./in. <sup>2</sup> | <1.5  |
| Hydrocarbon type analysis:                    |       |
| Paraffins, vol. percent                       | 64.6  |
| Naphthenes, vol. percent                      | 22.0  |
| Olefins, vol. percent                         | 0.8   |
| Aromatics, vol. percent                       | 12.6  |
| Distillation:                                 |       |
| Initial boiling point, ° F.                   | 237   |
| 10%                                           | 292   |
| 35 50%                                        | 327   |
| 90%                                           | 374   |
| End point                                     | 406   |
| Octane No. (Micro) Research Method:           |       |
| Clear                                         | 22.2  |
| 40 +3 cc. TEL/gal.                            | 47.2  |

Each of the runs was carried out in a fixed fluid-bed reaction system using a powdered molybdena-on-alumina reforming catalyst. The catalyst consisted of 10.8 percent by weight molybdenum trioxide impregnated on alumina coprecipitated with about 5 percent silica. Before starting the series of runs the catalyst was calcined overnight in air at 1000° F. and for three hours at 1100° F. The catalyst was then treated in accordance with the invention as described in the specific example below.

#### Example

The calcined catalyst was reduced with purified hydrogen containing 4.7 mol percent steam at a temperature of 900° F., a pressure of 250 pounds per square inch gauge and a linear gas velocity of 0.1 foot per second for one hour. Then a mixture of the Kuwait naphtha described above and hydrogen in proportions of 5000 standard cubic feet of hydrogen per barrel of naphtha was charged to the fixed bed fluidized catalyst. The hydrogen used during this period was substantially free of steam or other oxygenic substances. It contained less than about 0.01 mol percent steam. The reaction conditions included an average temperature of 903° F., a 55 pressure of 250 pounds per square inch, and a space velocity of 1.0 liquid volume of naphtha per volume of catalyst per hour. The mixture of hydrocarbons and hydrogen was charged to the catalyst bed for a period of three hours. During the first hour of the three hour 60 period, all operating variables were lined out. The second two hours was the on-stream period during which products were collected.

At the end of this first run, the catalyst was flushed with hydrogen, depressured, flushed with nitrogen, and then regenerated to remove coke deposits. The regen-

eration was carried out by flowing air through the catalyst for one hour at temperatures in the range of 900° to 1100° F. to burn off the deposited coke.

The catalyst described in the example was then used in a number of other runs. Certain of the runs followed the method of the invention, using in the reduction stage hydrogen that contained a substantial proportion of steam. The other runs followed a conventional method, using for both the reduction and on-stream stages hydrogen that contained less than 0.01 percent steam. Some of the runs, either by the method of the invention or by the conventional method, used the reduction temperature of 900° F., described in the example above. Other runs by both methods used a reduction temperature of 1050° F. The specific operating conditions for the reduction stage and the hydroreforming stage for each of the runs are given in Tables I through VIII below. The tables also give results for each run in terms of yield and octane ratings of gasoline products.

TABLE I

| Run                                        | Hydrogen with steam for reduction |       | Hydrogen without steam for reduction |       |
|--------------------------------------------|-----------------------------------|-------|--------------------------------------|-------|
|                                            | 1                                 | 2     | 3                                    | 4     |
| <b>Reduction conditions:</b>               |                                   |       |                                      |       |
| Temperature, ° F.                          | 900                               | 900   | 900                                  | 900   |
| Steam content of hydrogen, mol percent     | 4.7                               | 4.9   | <0.01                                | <0.01 |
| <b>Processing conditions:</b>              |                                   |       |                                      |       |
| Temperature, ° F.                          | 903                               | 903   | 906                                  | 901   |
| Pressure, p.s.i.g.                         | 250                               | 250   | 250                                  | 250   |
| Space velocity, vol.vol./hr.               | 1.0                               | 1.0   | 1.0                                  | 1.0   |
| H <sub>2</sub> :naphtha ratio, s.c.f./bbl. | 5,000                             | 4,900 | 5,000                                | 5,100 |
| <b>C<sub>5</sub>+</b> product data:        |                                   |       |                                      |       |
| Yield, percent by volume                   | 68.7                              | 68.2  | 67.5                                 | 68.6  |
| Octane number, micro research (clear)      | 93.6                              | 92.9  | 92.1                                 | 91.6  |

In Table I the yields and octane numbers are given for C<sub>5</sub>+ gasoline product. These data were obtained by standard calculations which adjusted the data obtained by analysis of the raw gasoline product to data for a debutanized gasoline, free of butanes and lighter hydrocarbons. Table I shows that the use of steam during the catalyst reduction at 900° F. in runs 1 and 2 substantially improved the yield-octane relationship of the C<sub>5</sub>+ product. Comparing runs 1 and 4 in which yields were about equal, the octane number of the clear C<sub>5</sub>+ product was 93.6 for our process (run 1) using steam in the hydrogen reduction stage and 91.6 for the conventional process (run 4) using dry hydrogen for reduction. This increase of 2.0 points of octane rating is, of course, very significant at this high octane level. Comparing runs 2 and 3, it is seen that the difference in octane ratings of the product is less than between runs 1 and 4 but that the yield difference is greater. Very clearly our process has improved the yield-octane relationship.

TABLE II

| Run                                        | Hydrogen with steam for reduction |       | Hydrogen without steam for reduction |       |
|--------------------------------------------|-----------------------------------|-------|--------------------------------------|-------|
|                                            | 5                                 | 6     | 5                                    | 6     |
| <b>Reduction conditions:</b>               |                                   |       |                                      |       |
| Temperature, ° F.                          | 900                               | 900   | 900                                  | 900   |
| Steam content of hydrogen, mol percent     | 4.7                               | <0.01 | 4.7                                  | <0.01 |
| <b>Processing conditions:</b>              |                                   |       |                                      |       |
| Temperature, ° F.                          | 903                               | 906   | 903                                  | 906   |
| Pressure, p.s.i.g.                         | 250                               | 250   | 250                                  | 250   |
| Space velocity, vol.vol./hr.               | 1.0                               | 1.0   | 1.0                                  | 1.0   |
| H <sub>2</sub> :naphtha ratio, s.c.f./bbl. | 5,000                             | 5,000 | 5,000                                | 5,000 |
| <b>C<sub>4</sub>+</b> product data:        |                                   |       |                                      |       |
| Yield, percent by volume                   | 80.6                              | 79.4  | 80.6                                 | 79.4  |
| Octane number, micro research (clear)      | 94.5                              | 93.2  | 94.5                                 | 93.2  |

Table II gives a comparison of a run by our method and a run following conventional procedure. Results are reported on the basis of the C<sub>4</sub>+ or depropanized gasoline product. Run 5, in which the catalyst was reduced with hydrogen containing steam in the method of the invention, produced a C<sub>4</sub>+ gasoline of greater yield and higher clear octane rating than run 6, carried out by conventional procedure with catalyst reduction with hydrogen containing no steam.

TABLE III

| Run                                        | Hydrogen with steam for reduction |       | Hydrogen without steam for reduction |       |
|--------------------------------------------|-----------------------------------|-------|--------------------------------------|-------|
|                                            | 7                                 | 8     | 7                                    | 8     |
| <b>Reduction conditions:</b>               |                                   |       |                                      |       |
| Temperature, ° F.                          | 900                               | 900   | 900                                  | 900   |
| Steam content of hydrogen, mol percent     | 5.4                               | <0.01 | 5.4                                  | <0.01 |
| <b>Processing conditions:</b>              |                                   |       |                                      |       |
| Temperature, ° F.                          | 901                               | 901   | 901                                  | 901   |
| Pressure, p.s.i.g.                         | 250                               | 250   | 250                                  | 250   |
| Space velocity, vol.vol./hr.               | 1.0                               | 1.0   | 1.0                                  | 1.0   |
| H <sub>2</sub> :naphtha ratio, s.c.f./bbl. | 5,200                             | 5,100 | 5,200                                | 5,100 |
| <b>10 RVP product data:</b>                |                                   |       |                                      |       |
| Yield, percent by volume                   | 77.1                              | 74.5  | 77.1                                 | 74.5  |
| Octane number, micro research (clear)      | 93.5                              | 92.7  | 93.5                                 | 92.7  |

Table III gives a comparison of a run by the method of the invention and a run by conventional procedure on the basis of the yield and octane rating of the unleaded gasoline product adjusted to a Reid vapor pressure of 10 pounds per square inch by adding butanes. The product for our process, run 7, is superior both in yield and octane rating. The yield advantage is 2.6 percentage points and the octane advantage 0.8 point at a high octane level.

TABLE IV

| Run                                        | Hydrogen with steam for reduction |       | Hydrogen without steam for reduction |       |
|--------------------------------------------|-----------------------------------|-------|--------------------------------------|-------|
|                                            | 9                                 | 10    | 9                                    | 10    |
| <b>Reduction conditions:</b>               |                                   |       |                                      |       |
| Temperature, ° F.                          | 900                               | 900   | 900                                  | 900   |
| Steam content of hydrogen, mol percent     | 5.4                               | <0.01 | 5.4                                  | <0.01 |
| <b>Processing conditions:</b>              |                                   |       |                                      |       |
| Temperature, ° F.                          | 901                               | 906   | 901                                  | 906   |
| Pressure, p.s.i.g.                         | 250                               | 250   | 250                                  | 250   |
| Space velocity, vol.vol./hr.               | 1.0                               | 1.0   | 1.0                                  | 1.0   |
| H <sub>2</sub> :naphtha ratio, s.c.f./bbl. | 5,200                             | 5,000 | 5,200                                | 5,000 |
| <b>10 RVP product data:</b>                |                                   |       |                                      |       |
| Yield, percent by volume                   | 77.1                              | 74.2  | 77.1                                 | 74.2  |
| Octane number, micro research (+3 cc. TEL) | 100.4                             | 100.0 | 100.4                                | 100.0 |

<sup>1</sup> Performance number.

Table IV gives a comparison of our process and the conventional process on the basis of the yield and octane rating of the gasoline product adjusted to a 10 pound Reid vapor pressure and containing 3 cc. of tetraethyl lead per gallon. The octane rating for the product of our process, run 9, is substantially better and the yield is about 3 percentage points higher than that of the conventional process, run 10.

Tables I through IV show that the advantages for our process are not limited to any particular way of measuring results. The results on four different standard methods of calculating the product yield and octane rating show our process superior in every case. Tables V through VIII below record the results of runs in which the reduction temperature was 1050° F. In these runs the catalyst, after reduction at 1050° F., was cooled to the run temperature of about 900° F. in the presence of the hydrogen containing steam or the dry hydrogen used in the reduction. The cooling required about 30 minutes. Specific conditions and results for each run are given in the tables.

TABLE V

| Run                                       | Hydrogen with steam for reduction |       | Hydrogen without steam for reduction |       |
|-------------------------------------------|-----------------------------------|-------|--------------------------------------|-------|
|                                           | 11                                | 12    | 13                                   | 14    |
| Reduction conditions:                     |                                   |       |                                      |       |
| Temperature, ° F                          | 1,050                             | 1,050 | 1,050                                | 1,050 |
| Steam content of hydrogen, mol percent    | 4.7                               | 2.0   | <0.01                                | <0.01 |
| Processing conditions:                    |                                   |       |                                      |       |
| Temperature, ° F                          | 901                               | 902   | 898                                  | 901   |
| Pressure, p.s.i.g.                        | 250                               | 250   | 250                                  | 250   |
| Space velocity, vol.vol./hr               | 1.0                               | 1.0   | 1.0                                  | 1.0   |
| H <sub>2</sub> :naphtha ratio, s.c.f./bbl | 5,000                             | 5,000 | 5,100                                | 5,200 |
| C <sub>5</sub> + product data:            |                                   |       |                                      |       |
| Yield, percent by volume                  | 75.0                              | 72.5  | 73.5                                 | 72.2  |
| Octane number, micro research (clear)     | 89.9                              | 91.6  | 87.2                                 | 88.4  |

Table V gives a comparison of our process and the conventional process when a reduction temperature of 1050° F. is used. The comparison is based on the C<sub>5</sub>+ or debutanized clear gasoline product. The octane rating for the product of our process in run 12 was 3.2 points higher than that of the conventional process in run 14. The yield for our process was also somewhat greater. Table V shows that the advantages of our process are obtained with different steam concentrations in the hydrogen reduction stage. Run 11 used a steam concentration of 4.7 mol percent and run 12 a steam concentration of 2.0 mol percent. The octane-yield relationships of the products for both of these runs were superior to those for the conventional process runs 13 and 14.

TABLE VI

| Run                                       | Hydrogen with steam for reduction |    | Hydrogen without steam for reduction |  |
|-------------------------------------------|-----------------------------------|----|--------------------------------------|--|
|                                           | 15                                | 16 |                                      |  |
| Reduction conditions:                     |                                   |    |                                      |  |
| Temperature, ° F                          | 1,050                             |    | 1,050                                |  |
| Steam content of hydrogen, mol percent    | 0.5                               |    | <0.01                                |  |
| Processing conditions:                    |                                   |    |                                      |  |
| Temperature, ° F                          | 902                               |    | 898                                  |  |
| Pressure, p.s.i.g.                        | 250                               |    | 250                                  |  |
| Space velocity, vol.vol./hr               | 1.0                               |    | 1.0                                  |  |
| H <sub>2</sub> :naphtha ratio, s.c.f./bbl | 5,000                             |    | 5,100                                |  |
| C <sub>4</sub> + product data:            |                                   |    |                                      |  |
| Yield, percent by volume                  | 87.2                              |    | 84.0                                 |  |
| Octane number, micro research (clear)     | 91.2                              |    | 88.8                                 |  |

Table VI compares our process with the conventional process, using a reduction temperature of 1050° F., on the basis of the C<sub>4</sub>+ clear gasoline product. The table shows that our process produces advantages when a steam concentration as low as 0.5 mol percent is used in the reduction stage. Run 15, in which the catalyst was reduced with hydrogen containing 0.5 mol percent steam, yielded a C<sub>4</sub>+ product that was 3.2 percentage points better in yield and 2.4 points better in octane rating (clear) than the product of the conventional process, run 16.

TABLE VII

| Run                                       | Hydrogen with steam for reduction |    | Hydrogen without steam for reduction |  |
|-------------------------------------------|-----------------------------------|----|--------------------------------------|--|
|                                           | 17                                | 18 |                                      |  |
| Reduction conditions:                     |                                   |    |                                      |  |
| Temperature, ° F                          | 1,050                             |    | 1,050                                |  |
| Steam content of hydrogen, mol percent    | 2.0                               |    | <0.01                                |  |
| Processing conditions:                    |                                   |    |                                      |  |
| Temperature, ° F                          | 902                               |    | 901                                  |  |
| Pressure, p.s.i.g.                        | 250                               |    | 250                                  |  |
| Space velocity, vol.vol./hr               | 1.0                               |    | 1.0                                  |  |
| H <sub>2</sub> :naphtha ratio, s.c.f./bbl | 5,000                             |    | 5,200                                |  |
| 10 RVP product data:                      |                                   |    |                                      |  |
| Yield, percent by volume                  | 79.6                              |    | 79.0                                 |  |
| Octane number, micro research (clear)     | 92.6                              |    | 89.8                                 |  |

Table VII compares the product of our process when a reduction temperature of 1050° F. is used with that of the conventional process on the basis of the unleaded gasoline product adjusted to a 10 pound Reid vapor pressure. The product of our process, run 17, was somewhat superior in yield and had a clear octane rating of 2.8 points above that of the product of conventional process, run 18.

TABLE VIII

| Run                                       | Hydrogen with steam for reduction |    | Hydrogen without steam for reduction |  |
|-------------------------------------------|-----------------------------------|----|--------------------------------------|--|
|                                           | 19                                | 20 |                                      |  |
| Reduction conditions:                     |                                   |    |                                      |  |
| Temperature, ° F                          | 1,050                             |    | 1,050                                |  |
| Steam content of hydrogen, mol percent    | 4.7                               |    | <0.01                                |  |
| Processing conditions:                    |                                   |    |                                      |  |
| Temperature, ° F                          | 901                               |    | 901                                  |  |
| Pressure, p.s.i.g.                        | 250                               |    | 250                                  |  |
| Space velocity, vol.vol./hr               | 1.0                               |    | 1.0                                  |  |
| H <sub>2</sub> :naphtha ratio, s.c.f./bbl | 5,000                             |    | 5,200                                |  |
| 10 RVP product data:                      |                                   |    |                                      |  |
| Yield, percent by volume                  | 82.7                              |    | 79.0                                 |  |
| Octane number, micro research: +3 cc. TEL | 100.0                             |    | 99.0                                 |  |

Table VIII compares our process with the conventional process, using a reduction temperature of 1050° F., on the basis of the gasoline product adjusted to a 10 pound Reid vapor pressure and containing 3 cc. of tetraethyl lead per gallon. The product of our process, run 19, was superior in yield by 3.7 percentage points and in octane rating by 1.0 point as compared with the product of the conventional process, run 20.

The tables above show that our process gives a product with a yield-octane relationship superior to that of the product of the conventional process on any standard basis of calculation. The tables also show that the superiority of our process exists over a considerable range for the concentration of steam in the hydrogen used in the reduction stage of our process and over a considerable range for the temperature of reduction.

Obviously many modifications and variations of the invention as hereinbefore set forth may be made without departing from the spirit and scope thereof and therefore only such limitations should be imposed as are indicated in the appended claims.

We claim:

1. A catalytic reforming process which comprises reducing a reforming catalyst comprising molybdenum oxide with hydrogen containing an oxygenic gas selected from the group consisting of steam, oxygen and carbon dioxide in a concentration equal in oxygen content to 0.5 to 15 mol percent of steam and contacting the reduced catalyst under hydroreforming conditions with a charge comprising naphtha and hydrogen, said charge being substantially free of oxygenic gases.
2. A catalytic reforming process which comprises contacting a reforming catalyst comprising molybdenum oxide with hydrogen containing an oxygenic gas selected from the group consisting of steam, oxygen and carbon dioxide in an amount equal in oxygen content to 0.5 to 15 mol percent of steam at a temperature from 850° to 1200° F., and contacting the resulting catalyst under hydroreforming conditions with a charge comprising naphtha and hydrogen, said charge being substantially free of oxygenic gases.
3. A hydroreforming process which comprises reducing a catalyst comprising molybdenum oxide with hydrogen containing a gas selected from the group consisting of steam, oxygen and carbon dioxide in a concentration equal in oxygen content to 0.5 to 5 mol percent of steam, at a temperature from 1000° to 1100° F. and a pressure above 50 pounds per square inch, and contacting the resulting reduced catalyst with a charge comprising naphtha and hydrogen in proportions of at least 500

cubic feet of hydrogen per barrel of naphtha, said charge being substantially free of oxygenic gases and said contacting being under hydroreforming conditions including the pressure used in reducing the catalyst and a temperature above 750° F.

4. A hydroreforming process which comprises reducing a regenerated reforming catalyst comprising molybdenum oxide supported on an alumina carrier with hydrogen containing from 0.5 to 5 mol percent steam at a temperature from 1000° to 1100° F. and a pressure above 50 pounds per square inch, contacting the resulting reduced catalyst in a reaction zone with a charge comprising a straight-run naphtha and hydrogen in proportions of from 1,000 to 20,000 cubic feet of hydrogen per barrel of said naphtha, said charge being substantially free of oxygenic gases and said contacting being under hydroreforming conditions including the pressure used in reducing the catalyst and a temperature above 750° F.

5. A catalytic reforming process which comprises in a reduction stage reducing a regenerated reforming cat-

15

10 5 alyst comprising molybdenum oxide with hydrogen containing an oxygenic gas selected from the group consisting of steam, oxygen and carbon dioxide in a concentration equal in oxygen content to 0.5 to 15 mole percent of steam and thereafter in a reforming stage

10 contacting under hydroreforming conditions a charge comprising naphtha and hydrogen, said charge being substantially free of oxygenic gases, with a body of catalyst consisting essentially of the reduced, regenerated catalyst reduced according to the procedure of said reduction stage.

## References Cited in the file of this patent

## UNITED STATES PATENTS

|           |              |               |
|-----------|--------------|---------------|
| 2,270,715 | Layng et al. | Jan. 20, 1942 |
| 2,274,988 | Matuszak     | Mar. 3, 1942  |
| 2,700,639 | Weikart      | Jan. 25, 1955 |
| 2,710,827 | Gornowski    | June 14, 1955 |
| 2,772,217 | Nicholson    | Nov. 27, 1956 |